

## UNITED STATES PATENT OFFICE.

EMILE BRONNERT, OF MULHOUSE, FRANCE.

## MANUFACTURE OF VISCOSE SILK.

No Drawing.

Application filed November 17, 1921. Serial No. 515,988.

*To all whom it may concern:*

Be it known that I, EMILE BRONNERT, a citizen of the Republic of France, and resident of Mulhouse, France, have invented 5 certain new and useful Improvements in the Manufacture of Viscose Silk; and I do hereby declare the following to be a full, clear, and exact description of the invention.

The present invention relates to an improvement of the process for the direct manufacture of the finest viscose silk by using baths containing a mixture of sulphuric acid and ammonium sulphate, such as disclosed in my U. S. Patent No. 1,419,714 of 15 June 13, 1922.

This patent relates to the use of a spinning bath containing sulphate of ammonium as well as sulphuric acid for making very fine viscose silk thread fibres like those disclosed 20 in my U. S. Patent No. 1,393,198, of Oct. 11, 1921, and comprises pre-determining the minimum limit of the concentration of acid in the following manner:

Assume the concentration of acid to be 25 expressed in grams per liter and the diameter of the thread or fibre in deniers; also assume that the minimum concentration C of acid for a given denier D has been ascertained, then the approximate minimum 30 concentration C<sub>1</sub> for any other or desired denier D<sub>1</sub> will be represented by the formula

$$C_1 = \frac{C\sqrt{D}}{\sqrt{D_1}}$$

In my above-mentioned Patent No. 1,419,714, is shown how this shall be interpreted with respect to the ammonium sulphate, in spinning baths containing sulphate 40 of alkali or alkaline earths and sulphuric acid; or in lieu of a bath containing sulphuric acid alone.

In employing such solutions of ammonium sulphate not only the free sulphuric acid, 45 but also the sulphuric acid contained in the ammonium sulphate itself must be considered, and it was found that two parts of sulphate of ammonia must be reckoned for one part of free sulphuric acid in the formula.

This enables fine spinning from any spinning apertures of the size customarily used, as described in my aforesaid Patent No. 1,393,198, and enables the calculation of the 55 minimum concentration of sulphuric acid to be determined for any denier number from

the concentration found to be good for any other denier number.

The present invention results in a cheapening of the cost of carrying out the process, on account of using a smaller quantity of the necessary ammonium sulphate.

Furthermore, the new proportions of the bath are strikingly adapted for an economic regeneration of the baths weakened during 65 spinning, as described in my U. S. Patent 1,376,671 of September 7, 1920.

In the spinning of viscose in acidulated ammonium sulphate baths a certain amount of sodium sulphate is of course formed, the 70 smaller part of which remains in the spinning bath and the greater part is carried away with the fibre in and on which it is formed.

By systematically rinsing or scouring the 75 fibres with dilute sulphuric acid and adding the rinsing solution to the spinning bath after concentration by evaporation, a condition of equilibrium in salts is easily attained, and which has been found to be very 80 advantageous.

The necessary minimum concentration of the acid or of the ammonium salt component has to be adjusted for each titre.

In spinning fibres of two deniers, for example, a bath of the following composition is gradually reached, which by the constant addition of only a little ammonium salt and the necessary quantity of sulphuric acid, which is supplied with the salt and as concentrated rinsing solution above referred to, it is easy to keep the bath as constant as necessary for good spinning. The product will dye uniformly, and is of uniform physical characteristics.

The composition gradually reached is—

|                   | Grams. |
|-------------------|--------|
| Sulphuric acid    | 260    |
| Ammonium sulphate | 200    |
| Sodium sulphate   | 300    |

95

100

Obviously the proportions of the two salts are not rigidly fixed; for example, a certain amount of magnesium sulphate may also be added, provided the concentration of acid is adjusted to the degree of fineness required.

The threads spun from such a bath, containing not only sulphuric acid and ammonium sulphate but also the above mentioned sodium sulphate no longer have the characteristic round cross section of threads spun in baths containing only sulphuric acid and ammonium sulphate. Their cross-sec-

105

110

tion is changed to the well known irregular star-like or ribbon-like cross section with serrated or indented contours.

Fibres spun in such baths possess the property of shrinking very little when drying, a particularly valuable property in the wholesale production of loose fibres, as the troublesome drying under tension is eliminated.

10 I claim—

1. Process of manufacturing threads of any deniers below six deniers from raw viscose, which comprises forcing viscose through openings of a diameter considerably larger than the diameter of the thread to be spun in the case of viscose of normal fluidity, into a bath containing sulphuric acid, ammonium sulphate and sodium sulphate, the minimum concentration of the acid component of which bath is inversely

proportional to the square root of the denier numbers of the thread desired and the amount of acid per unit volume of said bath, reckoning the ammonium sulphate as equivalent to half its weight of sulphuric acid, is not allowed to fall below a certain minimum weight, the said minimum being experimentally determined for any one denier number.

2. The process of manufacturing very fine artificial silk fibres according to claim 1, wherein the experimentally determined minimum concentration of a thread of two deniers is taken as a standard of reckoning as furnished by a bath containing 200 grams of sulphuric acid, 200 grams of ammonium sulphate and 300 grams of sodium sulphate.

In testimony that I claim the foregoing as my invention, I have signed my name

EMILE BRONNERT.